

July 27, 1943.

W. H. SODERHOLM

2,325,079

## HEAT TREATMENT OF PROJECTILES

Filed June 11, 1941

3 Sheets-Sheet 1

Fig. 1.



July 27, 1943.

W. H. SODERHOLM

2,325,079

HEAT TREATMENT OF PROJECTILES

Filed June 11, 1941

3 Sheets-Sheet 2

Fig. 2.



Fig. 3.



Fig. 4.



Fig. 5.



Inventor

Walter H. Soderholm

By *EJ Kessenich & JW Church*

Attorneys

July 27, 1943.

W. H. SODERHOLM

2,325,079

HEAT TREATMENT OF PROJECTILES

Filed June 11, 1941

3 Sheets-Sheet 3

Fig. 6.



Inventor

Walter H. Soderholm

334 Gessnerich & Church

Attorneys

## UNITED STATES PATENT OFFICE

2,325,079

## HEAT TREATMENT OF PROJECTILES

Walter H. Soderholm, United States Army,  
Syracuse, N. Y.

Application June 11, 1941, Serial No. 397,651

13 Claims. (Cl. 148—10)

(Granted under the act of March 3, 1883, as  
amended April 30, 1928; 370 O. G. 757)

The invention described herein may be manufactured and used by or for the Government for governmental purposes, without the payment to me of any royalty thereon.

My invention relates to the heat treatment of ordnance projectiles whereby the fragmentation of the projectile is controlled.

Previously, in the manufacture of high explosive fragmentation shells it was necessary to produce sections of relative weakness in the shell body by grooving the outside or inside surfaces of the shell or by adding strengthening rings so as to obtain a controlled fragmentation of the shell. In many cases this required additional machining operations on the blank shell or required an elaborate casting or forging. In any event additional metal was required over and above that necessary to provide a shell strong enough to withstand normal handling. Due to the irregular portions on the outside surface, the shell would be needlessly impeded by air resistance, or due to the presence of the irregular portions on the inside of the shell, the amount of bursting charge which could otherwise be confined would be diminished. In order to provide a fragmentation shell from a blank shell it was necessary to add additional material, weight, expense and time; there is a marked reduction in the amount of material, weight, expense and time necessary to produce a fragmentation shell in accordance with my invention as will clearly appear from the description of my invention.

The fragmentation shell produced by the apparatus and method described herein is described and claimed in my divisional application, Serial No. 413,306 filed October 2, 1941.

An object of my invention is to provide apparatus for furnishing a high explosive projectile which has strengthened portions or zones incorporated within the body of the projectile material.

Another object of my invention is to provide apparatus for heat treating zones or portions of the projectile material whereby subsequent fragmentation of the projectile is controlled.

Another object of my invention is to perform a heat treatment on a high explosive projectile so that portions on the inside surface or outside surface of the projectile may be strengthened.

Another object of my invention is to provide an arrangement of induction heating coils and quenching ducts for heat treating a high explosive projectile whereby its fragmentation may be controlled.

Another object of my invention is to provide an

arrangement whereby relative portions of the body of a high explosive projectile are strengthened without resorting to machining or elaborate forging operations.

Another object of my invention is to provide apparatus for furnishing a fragmentation controlled projectile body at a smaller manufacturing cost and with less time consumption than those heretofore existing.

Another object of my invention is to provide apparatus for furnishing a fragmentation controlled projectile shell which has a smooth outside surface and also a smooth inside surface so that the minimum air resistance is offered to the projectile in flight and a maximum amount of bursting charge may be incorporated within the shell.

Another object of my invention is to provide apparatus for furnishing a fragmentation controlled shell which requires no additional rings or grooves to be formed on the cylindrical surfaces of the projectile shell to produce a controlled fragmentation.

Another object of my invention is to provide apparatus for furnishing a fragmentation controlled shell of relatively light weight.

The nature and objects of my invention will be clearly revealed in the following description and accompanying drawings wherein:

Fig. 1 represents the heating coil and quenching duct arrangements disposed on the outside and inside of the shell and means for selectively controlling the energization of the heating coils.

Fig. 2 discloses the arrangement of strengthened portions when the outside heating coils only were energized.

Fig. 3 discloses the arrangement of strengthened portions when the inside heating coils only were energized.

Fig. 4 discloses the arrangement of strengthened portions when both the inside and outside heating coils were energized.

Fig. 5 discloses a view taken on line 5—5 of Fig. 1.

Fig. 6 discloses a modification in which nozzles are mounted on the spool-shaped centrally disposed spacer members.

Fig. 7 discloses a gas flame arrangement for heat treating the shell.

In this particular instance my invention is shown in relation to an antiaircraft shell and might be applied before or after the "nosing in" operation has been performed on the shell; it is understood however that my invention is not limited exclusively to the particular type of shell

disclosed and might be applied to other ordnance projectiles so as to control their fragmentation.

Reference is made to the drawings wherein like numerals indicate like parts. The shell 10 is held in the heat treatment apparatus on the base plate 17 by gravity and in centered relationship to the heat treatment apparatus by the circular projection 11. Magnetic induction coils 12 are equally spaced within the shell and magnetic induction coils 13 are equally spaced surrounding the shell and on the same horizontal planes with the inner coils 12. The inner coils are spaced by spool-shaped members 14. The entire inner column of coils 12 and spacers 14 is supported on the washer 15 which is held against downward movement by the fixed flange 15'. The coils 12 may be adjusted for height by making use of the threaded connection 18 between the tube 16 and base plate 17. The centrally disposed tube 16 has an indentation 19 on its outer surface which serves to prevent rotation of the spacers 14 with respect to the tube and also to serve as a conduit for the individual coil leads 20 which might be threaded through a cable 20'. Each spacer 14 has a transverse hole 21 through which the leads from one coil pass and also lugs 22, Fig. 5, which are adapted to cooperate with the inside corners 23 of the centrally disposed member 16 so as to prevent relative rotation.

A hole 24 in the base plate 17 provides an exit for the coil leads.

The upper end of tube 16 is provided with a small opening 27 so as to allow passage of the quenching fluid which might be water or oil. Holes 25 in the centrally disposed conduit 16 are arranged so that they are aligned with the holes 26 in spacers 14 thus allowing most of the quenching fluid to be squirted through those holes in the most effective regions. The holes 25, 26, 27 are graduated in size so that practically a uniform spray is produced in the interior of the shell; the holes are enlarged more and more as the distance from the source of supply is increased so as to compensate for the pressure drop of the quenching fluid. If desired, nozzles 28 may be mounted over each quenching fluid opening in the spacers as shown in the modification in Fig. 6 in order to more positively direct the quenching liquid to the heated shell surface although the addition of such nozzles is not deemed vitally necessary to carry out my invention.

The coils 13 are spaced by the circular channel shaped members 29 which have circumferentially disposed holes 40 aligned with holes 30 in the jacket 31. The row of coils 13 is supported on the washer-shaped member 32 which is held against downward movement by a fixed bracket 33. The jacket 31 has a recess 34 which serves as a conduit for the leads of coil 13; the inner edges 35 and 36 cooperate with lugs 37 and 38 on the circular channel-shaped members 29 so as to prevent relative rotation between members 29 and jacket 3.

The coil mounting structures for coils 12 and 13 are preferably of non-metallic material and it is desirable that the shell metal itself is the only metallic material through which the flux from coils 12 and 13 is caused to pass.

The jacket 31 is supplied with quenching fluid 70 which passes through the tubular opening 41. Gate valves 42 and 43 serve to limit the flow of quenching fluid to the inner and outer parts of the shell respectively.

The holes 30 may not all have the same diam-

eter but some of them may be enlarged so that equal amounts of quenching fluid will be discharged through all the holes. Nozzles similar to the ones shown in Fig. 6 may be mounted in relation to each opening 40 so as to serve as more positive directing means for the quenching fluid.

All of the quenching fluid must pass through a magnetically operated valve 44. Magnetically operated valves per se are well known in the fluid distribution art and for that reason the particular structure of this valve is not disclosed. The valve is of the type in which movement of the magnetic member 45 upon energization of solenoid winding 46 opens the valve 44 to allow a flow of fluid; upon deenergization of winding 46 the valve 44 is biased by means not shown so as to close the valve. The coil 46 is energized from a battery 47 through a single pole, double throw switch 48 which has one set of terminals to which no wires are connected.

The leads 20 from the inner coils pass through the opening 24 to a junction box 49 and the leads 50 from the outer coils which are threaded through a cable 50' pass through the opening 51 to the junction box 52.

The inner or outer coils 12 or 13 may be connected in series or in parallel at the corresponding junction box or in any other manner desired. When the coils 12 or 13 are connected in series with one another then the net effect of the component coils 12 or 13 is to form a coil proper with each coil 12 or 13 a component of the coil proper. The coils might be connected with respect to one another so that the same amount of current does not pass through each one of the coils if it is desired to produce compensating effects. Variable resistors 53 and 54 serve to control the amount of current flowing to the coils 12 and 13 respectively.

The double pole, double throw switch 55 serves to energize the leads 50 from an alternating current source 56 through transformer  $T_1$  and leads 59. Two terminals of the switch 55 are left unconnected as indicated in Fig. 1.

The double pole, double throw switch 57 serves to energize the leads 20 from the alternating current source 56 through transformer  $T_2$  and leads 58. Two terminals of the switch 55 are left unconnected as indicated in Fig. 1.

As a precautionary measure the double throw switches 48, 55, and 57 may be interlocked (not shown) so that switch 48 is prevented from being closed when either switch 55 or switch 57 is closed; this would prevent the shell being needlessly cooled and heated at the same time.

It is obvious that the inner and outer coils may be individually or simultaneously energized so that at the election of the operator inner rings of the shell material may be heated or the outer rings of the shell material may be heated or else the inner and outer rings of the shell material may be heated simultaneously. A subsequent rapid cooling of the heated parts will produce a hardening of the material which was heated so that the shell has hardened portions as indicated in the drawings. Fig. 2 discloses the result obtained when the outside heating coils were energized; the dotted portions signify the hardened portions. Fig. 3 discloses the result obtained when the inside heating coils were energized and the dotted portions signify the hardened portions.

Fig. 4 discloses the result obtained when both the inside and outside coils were energized and

the dotted portions signify the hardened portions.

It is fundamental that an increase in hardness in shell material is accompanied by an increase in tensile strength so that for the purpose of this specification the terms connecting increase in hardness and increase in tensile strength may be used interchangeably.

In operation, the operator performs the following steps:

1. (a) Closes switch 55 or (b) switch 57 or (c) switch 55 and switch 57, depending upon the desired location of the hardened zones,
2. Opens all the switches which were closed in step 1, and then
3. Closes switch 48 to cool the material.

The shell material is heated due to eddy currents and/or hysteresis losses in the shell material itself. The heating is local in effect and is necessarily generated in that region through which the flux passes in accordance with well-recognized principles.

High frequency currents may be used to great advantage in producing a heated zone near the surface of the shell material. The alternating flux through the coils 12 and 13 causes an alternating flux to pass through the shell material; the magnitude of the eddy currents produced in the shell material is in proportion to the frequency of the alternating current and these eddy currents set up magnetic fields of their own which tend to decrease the distance which the coil flux penetrates the shell material. The above phenomenon is commonly referred to as eddy current shielding and is made of advantage in producing a heated zone near the surface of the material. It is highly desirable that those portions which are to be hardened be heated above the hardening temperature very quickly and also quenched very quickly; otherwise the heat generated would have time in which to diffuse into the body of the material due to the good heat conduction of the body and instead of having sharply defined hardened bands in the shell there would be a hardening of that material which is not desired to be hardened. The electrical control arrangement described allows rapid operation. The power supply and connected circuits should be of sufficient size and have sufficient regulation to cause the shell material to be heated to the quenching temperature in the shortest possible time thus assuring a minimum amount of heat diffusion to the surrounding material.

The electrical and magnetic apparatus disclosed serves as one of the means by which a heat treated fragmentation shell of the type described may be produced. The embodiment of my invention thus far described is my preferred embodiment and it is understood that other means may readily be suggested; for instance, the portions of the shell to be hardened may be supplied by heat from a sharply defined gas flame which is movable with respect to the shell as in Fig. 7. In Figure 7, the shell 10 is held and rotated by a lathe chuck 90. Gas burners 112 and 113 supply heat to the inside and outside of the shell respectively. As the shell is rotated rings of the shell material will be heated above the temperature of its surrounding material. The flow of gas to the burners is controlled by the valves 142, 143 and 144. The flow of quenching fluid is controlled by valve 145. The valves 144 and 145 may be interlocked by means well known

in the art. The auxiliary valve 146 serves as an exit for any quenching fluid remaining in the gas pipes after the quenching operation.

It is to be understood that my invention is not limited to the production of a fragmentation shell of the type disclosed but my invention in its broader aspects may be applied in the production of ordnance matériel wherein it is desired to produce different degrees of strength or hardness in portions of the ordnance matériel.

In general my invention may be applied in the production of hand grenades, time delay bombs, projectiles or other fragmentation body so as to control the uniformity of the particles which are fragmented by the bursting charge contained therein.

I claim:

1. In the art of producing a fragmentation controlled shell, the apparatus comprising more than two spaced coaxial coils adapted to partially encase the shell, orifices disposed between adjacent coils, means to project a stream of liquid through said orifices, means for maintaining the shell stationary with respect to the coils, and means for spacing said coils whereby rings of the shell material are heated when high frequency current is passed through the coils.

2. In the art of producing a fragmentation controlled hollow shell, the apparatus comprising more than two spaced coaxial coils adapted to be disposed within the interior portion of the shell and in close proximity thereto, orifices disposed between adjacent coils, means for projecting a stream of liquid through said orifices, means for maintaining the shell stationary with respect to the coils, and means for spacing said coils whereby rings of the shell material are selectively heated when high frequency current is passed through the coils.

3. In the art of producing a fragmentation controlled shell, the apparatus comprising more than two spaced coaxial coils adapted to partially encase the shell, means for producing a spray of liquid within the cylindrical space defined by the coils, means for maintaining the shell stationary with respect to the coils, and means for spacing said coils whereby rings of the shell material are selectively heated when high frequency current is passed through the coils.

4. In the art of producing a fragmentation controlled hollow shell, the apparatus comprising more than two spaced coaxial coils adapted to be disposed within the interior portion of the shell and in close proximity thereto, means for producing a spray of liquid within the space surrounding the coils, means for maintaining the shell stationary with respect to the coils, and means for spacing said coils whereby rings of the shell material are selectively heated when high frequency current is passed through the coils.

5. In the art of producing a fragmentation controlled shell, the apparatus comprising more than two spaced coaxial coils adapted to partially encase the shell, means for maintaining the shell stationary with respect to the coils, and means for spacing said coils whereby rings of the shell material are selectively heated when high frequency current is passed through the coils.

6. In the art of producing a fragmentation controlled hollow shell, the apparatus comprising more than two spaced coaxial coils adapted to be disposed within the interior portion of the shell, means for maintaining the shell stationary with respect to the coils, and means for spacing said coils whereby rings of the shell material are selec-

tively heated when high frequency current is passed through the coils.

7. In the art of producing a fragmentation controlled hollow shell, the apparatus comprising a set of more than two spaced coaxial coils adapted to partially encase the shell, a set of more than two spaced coaxial coils adapted to be disposed within the interior portion of the shell and disposed coaxially with said first mentioned set, means for maintaining the first mentioned set stationary with respect to the shell, means for maintaining the second mentioned set stationary with respect to the shell and coaxial with the first mentioned set, means for spacing the coils of the first mentioned set whereby rings of the outer shell material are selectively heated when high frequency current is passed through the coils of the first mentioned set, and means for spacing the coils of the second mentioned set whereby rings of the inner shell material are selectively heated when high frequency current is passed through the coils of the second mentioned set.

8. In the process of producing a fragmentation body from a smooth surfaced body the steps which comprise, heating selected portions of the smooth surfaced body and then quickly quenching the selected portions, whereby fragmentation is controlled.

9. In the process of producing a fragmentation body from a hollow body having an outer smooth surface and an inner smooth surface, the steps which comprise heating selected portions of both smooth surfaces, and then quickly quenching the

selected portions so as to control the fragmentation of the body.

10. In the process of producing a fragmentation shell from a hollow shell having smooth cylindrical outer and inner walls, the steps which comprise heating selected portions of the inner and outer smooth cylindrical walls, and then quickly quenching the selected portions, whereby fragmentation is controlled.

11. In the process of producing a fragmentation shell from a hollow shell having smooth cylindrical inner and outer walls, the steps which comprise selectively heating ring-like portions of the inner and outer walls and then quickly quenching the heated portions.

12. The same as claim 7 and the plane of each coil of each set is coplanar with a corresponding coil of the other set.

13. The process of augmenting the fragmentation characteristics of a high explosive container formed of a ferrous metal of substantially the same composition throughout the surface area, which comprises, heating predetermined areas of the container at such a rate and to such a temperature as to permit hardening of areas of controlled depth of the container wall, terminating the heating when said areas attain the hardening temperature and chilling the areas so heated at such a rate as to increase the hardness of the same whereby the container walls are formed of areas of relatively high and low tensile strength.

WALTER H. SODERHOLM.